

## 1

3,476,616

**STAINLESS STEEL BARS AND RODS OF IMPROVED CROSS-SECTIONAL HARDNESS UNIFORMITY**  
Edward J. Dulis, Mount Lebanon Township, Allegheny County, Pa., assignor, by mesne assignments, to Crucible Inc., a corporation of Delaware  
No Drawing. Filed Sept. 1, 1966, Ser. No. 576,529  
Int. Cl. C21d 7/14

U.S. CL. 148—12

2 Claims

### ABSTRACT OF THE DISCLOSURE

This invention relates to bars or rods of metal having a face-centered-cubic crystal structure, such as austenitic stainless steel, and in particular, to bars or rods of such metal for use in automatic screw-making machinery or in other applications wherein the machinability of the metal is important. Still more particularly, the invention concerns bars or rods of the kind above-indicated that exhibit a relatively uniform hardness across the cross-sectional area thereof, and to a novel method of making such bars or rods.

### BACKGROUND OF THE INVENTION

In the as-annealed condition, bars or rods of austenitic stainless steel exhibit a relatively uniform hardness profile, ranging, for example, from 190 BHN at the edge to 170 BHN at the center. In that condition, however, long-time experience in commercial machining operations has shown that the steel is too soft to machine well in many instances because it is somewhat gummy. Hence, it has hitherto been the practice to cold-draw the steel at room temperature to the extent of about 6% reduction in cross-sectional area to increase the hardness to about 220 BHN at the midradius. This practice works the steel so that it imparts a relatively excessively hard surface (about 290 BHN). The cold-drawing operation raises the hardness of the center to about 200 BHN. Points between the center and the edge have hardness between those values. Now the hardness of the edge is undesirably high. The high surface hardness is related to lower lathe machinability rating and poorer chip rating as will be shown hereinbelow (see Table IV). The bar or rod is ground to remove a surface layer, for example, about 0.003 inch thick. After being ground, the bar or rod is still undesirably nonuniform in hardness across its cross-sectional area. Such, however, is the nature of the bars or rods of austenitic stainless steel now commonly on the market.

### DESCRIPTION OF THE INVENTION

In accordance with the invention, it has been discovered that if the bars or rods are heated to a temperature of about 200 to 500° F. before being subjected to a final drawing operation, much more favorable results are obtained. When this is done, it is possible to obtain rods that exhibit, for example, a hardness of 213 BHN at the center and about 250 BHN at the edge. This invention is of considerable importance to a manufacturer of such bars

## 2

and rods; if it is desired to produce a rod of a given predetermined diameter with a specified surface hardness limit, it is much easier to do so with the bars produced by practicing the method of the instant invention than with those of the prior art. The bars or rods of the prior art exhibit a sharp hardness gradient in the vicinity of their edges, and it sometimes happens that when the bar has been machined or ground to the desired dimensions, its surface hardness is unsatisfactory. As indicated above, this undesirable hardness gradient will be far less likely to occur with bars or rods made in accordance with the instant invention.

The present invention encompasses a method wherein face-centered-cubic crystal structured stainless steels are plastically deformed in a temperature range of about 200° F. to the recrystallization temperature, the latter temperature varying in accordance with the amount of deformation and the temperature. Basically, the mechanism involves the warm working of the face-centered-cubic austenite to impart a depth hardening by austenite deformation or by austenite deformation plus minimized deformation-transformation product. Thus, both the stably austenitic stainless steels, which remain completely austenitic after severe deformation at room temperature, and the unstably austenitic stainless steels, which undergo partial austenite deformation hardening and partial austenite-to-martensite transformation as a result of room-temperature transformation, are amenable to the development of improved hardness uniformity across the cross-section of bar sizes by the practice of the present invention. Significantly improved hardness uniformity can be achieved by warm plastic deformation of the various types of commercially used austenitic stainless steels. Studies were made on types 301, 304, 310, 316, 321 and 303 austenitic stainless steels. The results, presented hereinbelow in Table I, clearly show that a substantial improvement in cross-sectional hardness gradient is achieved in steels that are hardened by the plastic deformation of austenite only, as is shown by the lack of any magnetic response, a test that is commonly used to indicate the occurrence of transformation from austenite to deformation-induced martensite in the type 310 steel (J. B. Austin and D. S. Miller, "Magnetic Permeability of Some Austenitic Iron-Chromium-Nickel Alloys as Influenced by Heat Treatment and Cold Work," Trans. of the ASM, September 1940, pages 743-755, showed that type 310 does not form deformation-induced martensite even after severe deformation at room temperature). Also, type 301 steel, which is very likely to undergo transformation from austenite to deformation-induced martensite, has, in addition to the hardening mechanism of austenite deformation, a deformation-transformation-martensite formation, the latter reaction being partially suppressed by the warm deformation of the instant invention. Thus, regardless of whether the greater depth of uniform hardening attributable to warm drawing is related to austenite deformation only or to austenite deformation plus partial austenite to deformation-martensite formation, the degree of decrease in cross-sectional hardness gradient is clearly demonstrated.

TABLE I.—COMPOSITIONS OF ALLOYS USED FOR WARM DRAWING TRIALS

| Alloy | Bar Diameter (in.) | Composition (percent) |      |       |       |      |       |       |      |       |      |
|-------|--------------------|-----------------------|------|-------|-------|------|-------|-------|------|-------|------|
|       |                    | C                     | Mn   | P     | S     | Si   | Ni    | Cr    | Mo   | Zr    | Ti   |
| T301  | 1.00               | 0.03                  | 1.37 | 0.022 | 0.018 | 0.52 | 7.15  | 16.30 | —    | —     | —    |
| T304  | 1.00               | —                     | 1.27 | —     | —     | —    | 9.15  | 18.49 | —    | —     | —    |
| T316  | 1.00               | 0.06                  | 1.77 | 0.014 | 0.014 | 0.56 | 13.30 | 17.95 | 2.45 | 0.005 | —    |
| T321  | 1.00               | 0.042                 | 1.36 | —     | —     | 0.72 | 8.41  | 17.64 | 0.22 | —     | 0.57 |
| T310  | 0.750              | 0.05                  | 1.37 | 0.022 | 0.015 | 0.63 | 20.35 | 25.05 | —    | —     | —    |

| Alloy | Actual Reduction of area (percent) | Drawing Temp. (° F.) | Magnetic Responce | Hardness <sup>a</sup> (BHN) at Distance Below the Surface |           |           |           |           |           |           | Cross-Sectional Hardness Gradient (BHN) |
|-------|------------------------------------|----------------------|-------------------|-----------------------------------------------------------|-----------|-----------|-----------|-----------|-----------|-----------|-----------------------------------------|
|       |                                    |                      |                   | 0.500 in.                                                 | 0.375 in. | 0.282 in. | 0.250 in. | 0.188 in. | 0.130 in. | 0.094 in. |                                         |
| T301  | 8.4                                | RT                   | Very strong       | 233                                                       | 237       | —         | 250       | —         | 284       | —         | 307                                     |
|       | 9.1                                | 350                  | Strong            | 217                                                       | 218       | —         | 226       | —         | 239       | —         | 245                                     |
|       | 13.7                               | RT                   | Moderate          | 220                                                       | 223       | —         | 238       | —         | 254       | —         | 259                                     |
|       | 15.3                               | 350                  | Slight            | 217                                                       | 218       | —         | 221       | —         | 224       | —         | 228                                     |
|       | 13.4                               | RT                   | None              | —                                                         | 223       | 226.5     | —         | 233       | —         | 242.5     | 251                                     |
|       | 14.3                               | 350                  | do                | —                                                         | 221       | 223.5     | —         | 228       | —         | 233.5     | 238                                     |
| T310  | 25.2                               | RT                   | do                | —                                                         | 247       | 248.5     | —         | 255       | —         | 266.5     | 275                                     |
|       | 26.9                               | 350                  | do                | —                                                         | 237       | 237       | —         | 288.5     | —         | 244.5     | 250                                     |
|       | 15.5                               | RT                   | Moderate          | 222                                                       | 229       | —         | 234       | —         | 244       | —         | 250                                     |
|       | 16.2                               | 350                  | Slight            | 220                                                       | 222       | —         | 224       | —         | 229       | —         | 233                                     |
| T316  | 15.5                               | RT                   | Moderate          | 235                                                       | 238       | —         | 248       | —         | 268       | —         | 268                                     |
|       | 16.3                               | 350                  | do                | 218                                                       | 220       | —         | 225       | —         | 230       | —         | 228                                     |

<sup>a</sup> Diamond pyramid hardness values converted to BHN. Hardness results the average of five tests.

The invention finds use in the manufacture of bars, rods, etc., ranging in size from  $\frac{1}{4}$  in. to as high as 4 in., although most typically it is used in making rounds, hexes, squares and other shapes in the vicinity of  $\frac{1}{2}$  to 2 in.

The invention finds use in making bars or rods of any metal having an austenitic (face-centered cubic) crystal structure, including certain cobalt-base or nickel-base super-alloys, where hardness increase by cold work plus hardness uniformity are important (for example, for material for fastener applications), but it is most commonly useful with reference to the austenitic stainless steels of the 200 series and the 300 series. The new process is particularly useful with the free-machining grades of austenitic stainless steel, such as AISI type 303 and AISI type 303-SE stainless steel.

The temperature to which the steel is warmed before being cold drawn may, as indicated above, range from about 200° F. to 500° F., or possibly somewhat higher temperatures up to about 800° F. may be used, but in any event I use a temperature below the recrystallization and the carbide-precipitation temperatures of the metal. Problems related to carbide precipitation, such as reducing corrosion resistance (particularly intergranular corrosion resistance), occur during heating in the range about 900 to 1300° F., so that this temperature range is avoided. Apart from making it somewhat easier to effect heavier draws, the use of higher temperatures within that range has little to recommend it in comparison with the use of lower temperatures in the range. In addition, at higher temperatures, there may be difficulty in finding a lubricant of adequate stability.

The extent of reduction in area of the bar or rod as a result of the drawing operation may range from about 3% to about 20%. Smaller reductions tend to increase the center and mid-radius hardness considerably less than larger reductions. Hence, for most purposes, it is preferred to use a draw that reduces the cross-sectional area by about 5 to 8%.

As a specific example of the practice of the invention, samples from a commercial heat of free-machining austenitic stainless steel of the following composition were investigated: 0.09% carbon, 3.20% manganese, 0.019%

35 phosphorus, 0.33% sulfur, 0.51% silicon, 7.82% nickel, 17.99% chromium, 0.05% vanadium, 0.20% molybdenum, 0.17% copper, balance iron. The steel was cast into a commercial-sized ingot, hot-rolled to a cross section of about 1 in. round, and annealed. Upon being heated to 300° F. and then being warm-drawn to the extent of 5.17% reduction in area, the steel exhibited a center hardness of 205 BHN and an edge hardness of 247 BHN. For purposes of comparison, the same steel, drawn to the extent of 4.25% reduction in area at room temperature, exhibited a center hardness of 196 BHN and edge hardness of 275.5 BHN.

40 Further data relating to tests with the same steel and demonstrating the effect of the invention are presented in the following Table II.

TABLE II

| Draw Temper-ature | Reduc-tion in Area, Percent | BHN    |                      |            |                      |                 |  |
|-------------------|-----------------------------|--------|----------------------|------------|----------------------|-----------------|--|
|                   |                             | Center | $\frac{1}{4}$ Radius | Mid-Radius | $\frac{3}{4}$ Radius | 0.030 from Edge |  |
| R.T.              | 4.25                        | 196    | 196.5                | 200        | 220                  | 275.5           |  |
|                   | 10.95                       | 237    | 242                  | 257        | 288                  | 293             |  |
| 200° F.           | 4.53                        | 197    | 197.8                | 203        | 222                  | 256             |  |
|                   | 7.52                        | 213    | 216.4                | 222        | 235.5                | 250             |  |
| 300° F.           | 11.52                       | 231    | 231.5                | 237.5      | 251.6                | 260             |  |
|                   | 5.17                        | 205    | 205.5                | 206.8      | 220.5                | 247             |  |
| 400° F.           | 7.88                        | 215    | 215.5                | 217        | 240                  | 250             |  |
|                   | 11.67                       | 226    | 227                  | 230.5      | 244.5                | 261             |  |
| 500° F.           | 15.77                       | 240    | 241.8                | 248        | 257                  | 264             |  |
|                   | 5.35                        | 209    | 209                  | 214        | 230                  | 258             |  |
|                   | 7.88                        | 215    | 223.5                | 238        | 240                  | 248             |  |
|                   | 11.97                       | 231.5  | 232                  | 237        | 248.7                | 261             |  |
|                   | 16.01                       | 243.5  | 243.5                | 245.5      | 256                  | 261.5           |  |
|                   | 5.53                        | 200    | 200.5                | 204.8      | 220                  | 239             |  |
|                   | 8.42                        | 215    | 216                  | 220.5      | 234.5                | 247             |  |
|                   | 12.18                       | 232    | 233.2                | 238.3      | 252.5                | 258.5           |  |
|                   | 16.13                       | 243.5  | 243.6                | 248        | 256.7                | 261.5           |  |

70 Moreover, with respect to another commercial 15-ton heat of free-machining austenitic stainless steel consisting of 0.09% carbon, 1.68% manganese, 0.254% sulfur, 0.032% phosphorus, 0.40% silicon, 8.49% nickel, 17.12% chromium, 0.031% nitrogen, balance iron except for impurities, data were obtained that indicate the superiority in cross-sectional hardness uniformity and machinability of rods of austenitic stainless steel treated in accordance with the invention in comparison with cold-drawn rods of the same steel.

TABLE III

| Sample Number | Percent R.A. <sup>1</sup> | Draw Temp., °F. | Draw Speed, f.p.m. | Brinell Hardness Number<br>Distance below Surface (inch) |       |       |       |       | Machinability Rating            |                          |
|---------------|---------------------------|-----------------|--------------------|----------------------------------------------------------|-------|-------|-------|-------|---------------------------------|--------------------------|
|               |                           |                 |                    | 0.030                                                    | 0.125 | 0.250 | 0.375 | 0.500 | Lathe Mach. Rating <sup>3</sup> | Chip Rating <sup>4</sup> |
| 50            | ANN                       |                 |                    | 195                                                      | 183   | 171   | 175   | 163   | 101                             | 1                        |
| 51            | ANN                       |                 |                    | 178                                                      | 177   | 174   | 170   | 171   | 101                             | 1                        |
| 27            | 2 RT                      | 26              | 281                | 263                                                      | 236   | 226   | 218   | 213   | 94                              | 4-5                      |
| 11            | 2 RT                      | 50              | 293                | 259                                                      | 238   | 226   | 221   | 211   | 79                              | 5                        |
| 1             | 2 RT                      | 50              | 286                | 262                                                      | 235   | 226   | 219   | 219   |                                 |                          |
| 2             | 2 RT                      | 50              | 278                | 259                                                      | 232   | 222   | 219   | 223   | 82                              | 4                        |
| 44            | 2 RT                      | 50              | 286                | 260                                                      | 238   | 227   | 223   | 223   |                                 |                          |
| 30            | 3 RT                      | 70              | 286                | 262                                                      | 235   | 226   | 219   | 219   | 89                              | 5                        |
| 26            | 6                         | 200             | 26                 | 244                                                      | 234   | 221   | 215   | 214   | 92                              | 3-4                      |
| 16            | 6                         | 200             | 50                 | 249                                                      | 237   | 222   | 216   | 216   | 98                              | 4                        |
| 29            | 6                         | 200             | 70                 | 242                                                      | 233   | 221   | 215   | 213   | 99                              | 4                        |
| 28            | 6                         | 350             | 26                 | 243                                                      | 236   | 227   | 221   | 220   | 96                              | 4                        |
| 3             | 350                       | 50              | 240                | 229                                                      | 222   | 218   | 217   | 217   | 92                              | 3-4                      |
| 31            | 6                         | 350             | 50                 | 244                                                      | 226   | 212   | 209   | 209   | 93                              | 4                        |
| 23            | 6                         | 350             | 70                 | 245                                                      | 239   | 226   | 218   | 216   |                                 |                          |
| 24            | 6                         | 350             | 70                 | 246                                                      | 235   | 222   | 216   | 215   | 97                              | 4                        |
| 25            | 6                         | 350             | 70                 | 242                                                      | 227   | 217   | 213   | 212   | 98                              | 3                        |
| 33            | 10                        | 2 RT            | 50                 | 285                                                      | 267   | 252   | 246   | 246   | 83                              | 6                        |
| 32            | 10                        | 350             | 50                 | 247                                                      | 241   | 236   | 238   | 238   | 98                              | 4-5                      |

<sup>1</sup> Reduction of Area.<sup>2</sup> Room Temperature.<sup>3</sup> Higher rating indicates better machinability.<sup>4</sup> Higher chip rating indicates poorer chip.

Data with respect to further tests conducted with the steel consisting of 0.09% carbon, 3.70% manganese, 0.33% sulfur, 0.019% phosphorus, 0.55% silicon, 7.82% 40 and V. nickel, and 17.99% chromium, balance iron except for impurities, are presented in the following Tables IV

TABLE IV.—CROSS-SECTIONAL HARDNESS OF COLD AND WARM DRAWN TYPE 303 PLUS X

| Actual Percent Reduction of Area | Drawing Temperature, °F. | Brinell Hardness Number <sup>a</sup><br>Distance below the Surface |       |       |       |       | Cross-Sectional Hardness Gradient, BHN |
|----------------------------------|--------------------------|--------------------------------------------------------------------|-------|-------|-------|-------|----------------------------------------|
|                                  |                          | 0.030                                                              | 0.130 | 0.250 | 0.375 | 0.500 |                                        |
| 4.3                              | 1 RT                     | 286                                                                | 221   | 204   | 198   | 198   | 88                                     |
| 4.5                              | 200                      | 256                                                                | 223   | 208   | 204   | 202   | 54                                     |
| 5.2                              | 300                      | 262                                                                | 228   | 213   | 201   | 201   | 61                                     |
| 5.4                              | 400                      | 257                                                                | 230   | 214   | 209   | 209   | 48                                     |
| 5.4                              | 500                      | 258                                                                | 221   | 206   | 202   | 200   | 58                                     |
| 7.0                              | 1 RT                     | 262                                                                | 247   | 220   | 217   | 214   | 48                                     |
| 7.5                              | 200                      | 247                                                                | 238   | 224   | 218   | 218   | 29                                     |
| 7.9                              | 300                      | 246                                                                | 238   | 218   | 215   | 213   | 33                                     |
| 7.9                              | 400                      | 238                                                                | 233   | 221   | 217   | 217   | 21                                     |
| 8.4                              | 500                      | 244                                                                | 235   | 220   | 213   | 211   | 33                                     |
| 11.0                             | 1 RT                     | 290                                                                | 289   | 261   | 250   | 242   | 48                                     |
| 11.5                             | 200                      | 260                                                                | 258   | 247   | 238   | 234   | 26                                     |
| 11.7                             | 300                      | 258                                                                | 255   | 243   | 238   | 237   | 21                                     |
| 12.0                             | 400                      | 253                                                                | 250   | 244   | 236   | 236   | 27                                     |
| 12.0                             | 500                      | 260                                                                | 252   | 246   | 239   | 235   | 25                                     |
| 15.8                             | 300                      | 263                                                                | 257   | 248   | 242   | 240   | 23                                     |
| 16.0                             | 400                      | 262                                                                | 256   | 245   | 243   | 243   | 19                                     |
| 16.1                             | 500                      | 262                                                                | 258   | 250   | 243   | 243   | 19                                     |
| 0                                | ( <sup>b</sup> )         | 190                                                                | 183   | 184   | 186   | 185   | 7                                      |
| 6                                | ( <sup>c</sup> )         | 286                                                                | 255   | 236   | 225   | 222   | 64                                     |

<sup>a</sup> Hardness results are the average of five tests.<sup>b</sup> Room Temperature.<sup>c</sup> Mill Anneal.<sup>d</sup> Mill Drawn.

TABLE V.—DRILL AND LATHE MACHINABILITY OF WARM  
AND COLD DRAWN TYPE 303 PLUS X

| Actual Percent<br>Reduction<br>of Area | Drawing<br>Tempera-<br>ture, °F. | Drill<br>Machin-<br>ability<br>Rating <sup>a</sup> | Lathe Machinability |                             | 5  |
|----------------------------------------|----------------------------------|----------------------------------------------------|---------------------|-----------------------------|----|
|                                        |                                  |                                                    | Rating <sup>a</sup> | Chip<br>Rating <sup>b</sup> |    |
| 4.3                                    | Room                             | 103                                                | 94                  | 6                           |    |
| 4.5                                    | 200                              | 105                                                | 97                  | 2                           |    |
| 5.2                                    | 300                              | 104                                                | 97                  | 3                           |    |
| 5.4                                    | 400                              | 103                                                | 96                  | 3                           |    |
| 5.4                                    | 500                              | 105                                                | 96                  | 3                           |    |
| 7.0                                    | Room                             | 103                                                | 89                  | 4                           |    |
| 7.5                                    | 200                              | 104                                                | 89                  | 3                           | 10 |
| 7.9                                    | 300                              | 103                                                | 98                  | 2-3                         |    |
| 7.9                                    | 400                              | 104                                                | 96                  | 3                           |    |
| 8.4                                    | 500                              | 103                                                | 96                  | 3-4                         |    |
| 11.0                                   | Room                             | 101                                                | 81                  | 7                           |    |
| 11.5                                   | 200                              | 102                                                | 89                  | 5-6                         |    |
| 11.7                                   | 300                              | 103                                                | 86                  | 4                           |    |
| 12.0                                   | 400                              | 102                                                | 85                  | 4                           | 15 |
| 12.0                                   | 500                              | 102                                                | 90                  | 4-5                         |    |
| 15.8                                   | 300                              | 102                                                | 86                  | 4                           |    |
| 16.0                                   | 400                              | 103                                                | 85                  | 4                           |    |
| 16.1                                   | 500                              | 103                                                | 84                  | 5                           |    |
| 0                                      | (s)                              | 104                                                | 100                 | 1                           |    |
| 6                                      | (d)                              | 105                                                | 86                  | 7                           |    |

<sup>a</sup> Higher rating indicates better machinability.<sup>b</sup> Higher rating indicates a poorer chip.<sup>c</sup> Mill Anneal.<sup>d</sup> Mill Drawn.

While I have shown and described herein certain embodiments of the invention, I intend to cover as well any change or modification therein which may be made without departing from its spirit and scope.

## I claim:

1. In a method of making an austenitic stainless steel having a face-centered cubic crystal structure in the form of bars, rods, or wire, said bars, rods, or wire having improved cross-sectional hardness uniformity, the step comprising cold-working said bar, rod, or wire to the extent of a reduction in cross-sectional area of from 3% to 20% at a temperature between 200° F. and the recrystallization temperature of said steel.
2. A method as defined in claim 1, characterized in that said metal comprises a free-machining grade of austenitic stainless steel and is warm-worked to the extent of a reduction in cross-sectional area of between 5 and 8% at a temperature of 200° to 500° F.

## References Cited

## UNITED STATES PATENTS

|           |         |                 |        |
|-----------|---------|-----------------|--------|
| 2,716,080 | 8/1955  | Schwarz         | 148—12 |
| 2,767,837 | 10/1956 | Nachtman et al. | 148—12 |
| 2,924,543 | 2/1960  | Nachtman        | 148—12 |
| 2,924,544 | 2/1960  | Nachtman        | 148—12 |
| 3,001,897 | 9/1961  | Nachtman        | 148—12 |

L. DEWAYNE RUTLEDGE, Primary Examiner

W. W. STALLARD, Assistant Examiner

UNITED STATES PATENT OFFICE  
CERTIFICATE OF CORRECTION

Patent No. 3,476,616

November 4, 1969

Edward J. Dulis

It is certified that error appears in the above identified patent and that said Letters Patent are hereby corrected as shown below:

Columns 3 and 4, TABLE I, seventh column, line 3 thereof, "0.56" should read -- 0.66 --.

Signed and sealed this 21st day of April 1970.

(SEAL)

Attest:

Edward M. Fletcher, Jr.

Attesting Officer

WILLIAM E. SCHUYLER, JR.

Commissioner of Patents